

## UNITED STATES PATENT OFFICE.

WALTHER MATHESIUS, OF CHARLOTTENBURG, GERMANY.

## MANUFACTURE OF LEAD ALLOYS.

No Drawing.

Application filed October 21, 1922. Serial No. 596,129.

*To all whom it may concern:*

Be it known that I, WALTHER MATHESIUS, a German subject, residing in Charlottenburg, Germany, have invented a certain new 5 and useful Improved Manufacture of Lead Alloys, of which the following is a specification.

This invention relates to the manufacture of alloys of lead with more than one or 10 with three alkaline earth metals, calcium, barium and strontium in specified proportions.

It would be supposed that the simplest 15 method of making alloys of four metals would be to obtain the individual metals and then to mix them together directly for producing the alloy. In the present case, however, such a method is obviously impracticable. The manufacture of the individual 20 alkaline earth metals by electrolyzing their fused salts, in particular chlorides, has been successful hitherto only in the case of calcium.

It would appear to be possible to make 25 alloys of the individual alkaline earth metals with lead by using the molten lead as the cathode in electrolyzing the fused chloride. This operation, however, is unsatisfactory and uneconomical as the melting point of the 30 chloride is so high that the difference between the melting point and the boiling point of the chloride is so small that it is practically impossible in passing the current through the molten chloride to avoid 35 a rise of temperature towards or even up to the boiling point of the chloride. If this condition is attained not only is there a remarkable loss of current and other disturbance of the electrolytic operation, but 40 the operation is accompanied by much evolution of saline vapour which is very troublesome.

Further consideration of the matter shows 45 that when it is desired to introduce more than one, or all three, of the alkaline earth metals into the lead alloy so that all three chlorides, for instance, are used as the electrolyte, the operation becomes more favourable as the fusing point of the mixture is 50 considerably lower than that of the individual chlorides, so that the difference between melting point and vaporization point is essentially greater.

However, by this mode of working it is 55 difficult to obtain alloys of prescribed com-

position, for the metals pass into the lead cathode not in accordance with their proportion in the fused electrolyte but in a proportion which depends in the first place on their order of potential. Consequently 60 it is found that the fused electrolyte becomes impoverished in one metal and enriched in the other metal or metals.

The present invention relates to a mode of operation which renders it possible, in spite 65 of the above described normal behaviour of the mixture of salts when electrolyzed, to obtain alloys of all three alkaline earth metals with lead of predetermined composition, by using a molten lead cathode. 70

When a mixture of fused salts in given proportions is electrolyzed with the fused lead cathode the alloy which is first produced does not correspond with the composition of the mixture of salts. After a certain time, however, there is produced a condition of equilibrium and a further impoverishment or enrichment of the salt mixture does not occur. According to the invention 75 when this condition of equilibrium of the molten electrolyte is attained fresh portions of the salt mixture of predetermined composition may be added in small portions, whereupon the metals will separate exactly in the prescribed proportions and pass into the lead 80 in these proportions until the aforesaid condition of equilibrium is again attained.

At first therefore there is obtained a cathode alloy which in no way corresponds with the desired composition, but if in the course 90 of the operation a portion of the lead cathode is continuously removed and fresh lead is substituted for that portion the composition of the cathode alloy gradually changes until that desired is attained. 95

The amount removed and the amount added in unit time is in practice such as is suitable for the current strength.

When the form of the electrolytic bath and the magnitude of the current are suitable 100 it is possible to arrange a continuous discharging of the lead alloy and a continuous charging of the lead.

Without restricting myself to proportions, I will state that if it is desired to produce 105 an alloy containing lead as the major constituent, and containing equal proportions of calcium, barium and strontium, alloyed with said lead, a mixture of calcium chloride, barium chloride and strontium chloride con- 110

taining equal amounts of the three metals, can be used as the initial electrolyte. This mixture is fused on the lead bath which is to form the cathode, and an electric current is passed through the fused chlorides from an insoluble anode, to the lead cathode. The current density and the voltage, can both be a little greater than those ordinarily used in the electrolysis of fused calcium chloride. At first there is formed by electrolysis, a lead alloy containing somewhat more calcium, and somewhat less strontium than would correspond to equal amounts, and the electrolysis is continued until it is found that the composition of the fused bath remains substantially constant. When this condition has been reached, small additional quantities of the mixture of calcium chloride, barium chloride, and strontium chloride, containing equal amounts of the three metals, are added to the bath, about as fast as the constituents of the bath are being decomposed, by the electrolytic current. At the stage, when in addition of the mixed chlorides to the bath is commenced, the lead cathode can be drawn off and a new lead cathode substituted, after which the inflow of metallic lead and the outflow of the lead alloy, can be made continuous. It will be obvious that in place of starting with the mixture containing the above stated proportions of the three chlorides, it is possible to start with an electrolyte containing the fused chlorides, in about the proportions present in the electrolyte in the above example, at that stage where the addition of new amounts of the mixed chlorides is begun.

When the operation is on a large scale and of long duration, one can use the alloy produced up to the time when an equilibrium condition is attained without gross error in the total alloy, since when this incorrect alloy is mixed with a large quantity of the alloy of correct composition produced

later, the error in the composition of the whole alloy is practically reduced to zero.

I claim:—

1. The herein-described process of making lead alloys with more than one of the alkaline earth metals, by electrolysis of a fused mixture of salts of said alkaline earth metals, in contact with a lead cathode, which comprises, first electrolyzing a mixture of fused halogen salts of such alkaline earth metals, until the fused electrolyte has attained a condition of equilibrium in composition, wherein further electrolysis produces an alloy containing the alkaline earth metals in substantially uniform proportions to each other, and then adding to the electrolyte, successive small portions of a mixture of the salts of which the electrolyte is composed, the proportion of said alkaline earth metals in such mixture being that desired in the final alloy. 50
2. In the manufacture referred to in claim 1, the step of substantially continuously removing a part of the molten cathode and substantially continuously adding lead 60 to replace the alloy so withdrawn. 70
3. A process of preparing lead alloys containing more than one alkaline earth metal by electrolysis of a fused mixture of halogen salts of said alkaline earth metals, which 75 comprises the step of adding to a fused electrolyte composed of such haloid salts, wherein electrolysis produces an alloy containing the said alkaline earth metals in substantially the desired proportions, successive 80 small portions of a mixture of the salts of which the electrolyte is composed, the proportion of said alkaline earth metals in such mixture being that desired in the final alloy, while passing an electrolytic current through 85 said fused mass of salts, while in contact with a lead cathode.

In testimony whereof I have signed my name to this specification.

WALTHER MATHESIUS.